

1

3,179,575

METHOD OF PRODUCING SILVER LAYER ON  
NON-METALLIC ELECTRICALLY NON-CON-  
DUCTIVE SUPPORT

Cornelis Johannes Dippel and Hendrik Jonker, Eindhoven, Netherlands, assignors to North American Philips Company, Inc., New York, N.Y., a corporation of Delaware  
No Drawing. Filed July 11, 1960, Ser. No. 41,730  
Claims priority, application Netherlands, July 11, 1959,

241,195

10 Claims. (Cl. 204—38)

The invention relates to a method of manufacturing external, electrically conductive noble-metal layers on non-metallic, electrically non-conductive, at least superficially hydrophilized supports and to products manufactured by this method.

The term "noble-metal layers" is to be understood to mean herein not only layers having an uninterrupted surface of noble metal but also those having patterns, the portions of which may be discontinuous, for example, station-name dials for radio apparatus, ornamental objects, wiring patterns, circuit patterns, and so on.

According to the invention an external, electrically conductive noble-metal layer is produced on a non-metallic, electrically non-conductive, slightly hydrophilic or at least superficially hydrophilized support by activating said support by causing to take place on the support a reaction between a mercurous compound and agent capable of reacting with this mercurous compound, in the presence of water, to form metallic mercury, either by reduction or by disproportionating one of the reaction components being located in the support or at least in the surface thereof, and produce thereby an at least partly external, hardly visible layer of mercury germs on the support.

According to the invention, the hardly visible mercury germ layer is then treated with a non-stabilized noble metal intensifying bath comprising a non-stabilized aqueous solution of a metal compound more noble than copper and a reducing agent for the noble metal compound. By means of this step noble metal from the noble metal compound of this solution is reduced on the mercury germ layer and forms an electrically conductive noble metal layer having a resistance not greater than  $10^4$  ohms per square.

For the noble metal depositing bath there may be used the conventional baths for chemical silver deposition, but preferably use will be made of the purely physical developers usually intended for photographic purposes, since, in view of their great selectivity, they may be more easily controlled. Purely physical developers are distinguished from the so-called chemical silver deposition baths by the use of photographic reducing agents, i.e., compounds of which the reducing effect in the physical developer under the prevailing conditions, owing to the presence of the photographic metal germ image, is accelerated so that a sufficiently selective noble-metal deposition on this metal germ image is obtained. A frequently used physical developer is, for example, a solution of silver nitrate in water, to which is added metol, hydroquinone or p-phenylene-diamine. Such a developer contains, furthermore, usually substances to improve the preservability thereof or to control the speed of development, for instance, organic acids, buffer mixtures or substances reacting with the noble-metal compound, while forming a complex.

By the term "non-stabilized noble-metal intensifying bath" in the instant case is meant a noble-metal depositing bath, as defined supra, free of ionic surfactants added to prevent the noble-metal compound from being spontaneously reduced to metal in the aqueous solution.

2

Although it is possible to include, in the support during the manufacture thereof, the agent capable of reacting with the mercurous compound, in the presence of water, the activation of the support is usually carried out by treating the support surface, in order of succession, with an aqueous solution of an agent capable of reacting with a mercurous compound, in the presence of water, while separating out metallic mercury, and with an aqueous solution of a mercurous compound or conversely.

10 In order to keep the mercury layer formed uniform, it is advisable to wipe off the surface of the support after the first treatment, in order to remove adhering fluids. Particularly in the case in which the treatment with the mercurous compound reacting agent precedes and the support thus treated is afterwards treated with mercurous solution, better results are obtained, when the layer is dried after the first treatment.

15 Since the present invention is concerned with the manufacture of external, electrically conductive noble-metal layers by the intensification of external mercury germs, which lies on the support and which are obtained during the activation of the support by a reaction between a mercurous compound and an agent capable of reacting with this mercurous compound in the presence of water, to separate mercury metal, it will be obvious that care must be taken, by choosing the ratio between the concentrations of the mercurous compound solutions and the solutions of the mercurous reacting compound, that the reaction takes place indeed mainly at the surface of the support. A partial deposition in or below the surface is conducive to the adhesion of the noble-metal layer to the support. Irrespective of the order of succession in the two bath treatments, there can always be indicated, as far as the solubilities of the substances concerned permit doing so, a range of concentrations of the second bath at a given concentration of the first bath to obtain an at least partly external layer of mercury germs on the support, on which is to be deposited subsequently an external noble-metal layer with a resistance of not more than  $10^4$  ohms per square by treatment with the non-stabilized noble-metal intensifying bath. The limits of the said range may differ slightly with the individual compounds and supports. Therefore, the active range of concentrations of the second bath, with a given concentration of the first bath, must be fixed by a simple sequence of experiments, while the concentrations of the second bath are varied by a given factor (for example 2 to 3). It has been found that, at least when the support is dried intermediately between the two treatments, the concentration of the first bath must, as a rule, exceed that of the second bath. When the support is not dried between the treatments, materially higher concentrations of the first bath are to be employed than in the case of drying.

20 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 967

for decoration, electrical and electro-technical purposes. In the first case, the whole support surface is to be subjected to the activation. In the second case, the pattern may be applied previously by activating the surface in accordance with the pattern either directly by means of a printing technique or indirectly with the aid of a known mechanical or photographic masking technique, or the pattern may be obtained on the uninterrupted noble-metal layer finally obtained in accordance with the invention by etching away the redundant noble metal subsequent to covering by the noble-metal layer. All kinds of known methods of photo-engraving and graphics may be used in this case to apply a mask resisting the chemical treatment to be employed.

The external noble-metal layers obtained by the method according to the invention often have electric resistances which are many times higher than is calculated from the resistivity of the metal concerned in a compact state. By a thermal and/or chemical after-treatment and/or a mechanical polishing treatment the excessively high resistance of the layer can be considerably reduced, which is desirable for various electrical uses.

It is known (E. Raub, Z. Metallkunde 39, 33 (1948)) that with the electro-deposition of, for instance, silver metal, under certain conditions, non-metallic substances may, in addition, be included in the layer as impurities which affect particularly the electric resistance and the hardness of the layer. The high resistance of such a layer can be reduced by a thermal treatment in excess of a given temperature so that it approaches that value which can be calculated from the resistivity of the compact, pure metal.

In accordance with the invention, it has been found that heating of the external noble-metal layer obtained by intensification of an external layer of mercury germs to a temperature of at least 80° C. may result in a reduction of an excessively high resistance value of the layer. This heating may be performed, for instance, in a furnace with the aid of an infrared radiator, by electric current passing through the layer or by means of rinsing in a hot, chemically indifferent liquid (water or glycerol, for example). The desired effect is attained more rapidly as the temperature of the after-treatment is higher, but it must, of course, be considered that the material of the support constitutes a limit to the temperature that may be employed.

It has furthermore been found that the silver metal separated out in several, non-stabilized, purely physical developers has a more or less loose structure (so-called "black" silver), which can be rendered more compact by given chemical after-treatments (so-called "grey" silver). In this connection, reference is made to "C. K. Mees, The Theory of the Photographic Process," revised edition, 1954, page 753. As may be expected, the electric resistance is materially reduced. The phenomenon may be due to the flocculation of sols known from colloid chemistry. Any important reduction in electric resistance of the external silver layer obtained subsequent to intensification may be obtained by contacting this layer with an aqueous solution of one or more compounds separating off a hydrogen ion or an anion potential being determining with respect to the silver metal, for example, the chloride, bromide, iodide, thiocyanate, cyanide, sulphide, sulphite, thiosulphate or hydroxyl ion. For compounds separating off hydrogen or hydroxyl ions use may be made, not only of a diluted, non-oxidizing acid or a diluted base, but also of a solution of an acid or an alkali-reacting salt. As a rule, the resistance reducing effect is obtained more rapidly as the active compound is provided in a higher concentration, while with respect to the extent of the activity of the various anions the following sequence may be established:



As an alternative, the said reduction in resistance may be obtained by mechanical polishing.

For a great number of uses in the electrical and the electro-technical and the decoration fields it is necessary or desirable that the external, electrically conductive noble-metal layer obtained by the method according to the invention should be electro-chemically after-treated, which may be followed by a superficial chemical conversion or coloration.

To this end may be used, for example, electrolytic polishing, electrolytic deposition of metals, while using or not using an external current source, electrolytic coloration of the deposited metal or electrophoretic coating with a protective or insulating or photo-conductive and/or semi-conductive surface layer.

Moreover, a combination of various electro-chemical and/or chemical after-treatments is possible.

When the invention is to be used for the manufacture of metal patterns which are electrolytically intensified or electrophoretically coated the portions of the uninterrupted noble-metal layer not associated with the final pattern will be provided, preferably prior to the required treatment, with a resistant mask with the aid of a mechanical or photographic technique. The uncovered portions of the layer are then intensified or coated, while the uninterrupted layer provides a conductive contact between the parts of the final pattern. After removal of the mask, the pattern may be produced by etching away the redundant noble metal. The mask may, of course, also be applied subsequent to the electro-chemical after-treatment, the pattern being then obtained by etching away the metal of the uncovered portions of the layer. However, this is economically less advantageous. For the various uses there is furthermore a great choice among a number of known, mechanical after-treatments, which may be combined with the described after-treatments. A few, important, suitable after-treatments of this kind are, inter alia: mechanical polishing of the surface of the layer, application of a lacquer or varnish layer to the layer surface, embedding of the layer together with the support in an insulating envelope of thermo-hardening or thermo-plastic material, transfer of the layer, if desired together with the support, to a different support of high electric qualities, also of thermo-hardening or thermo-plastic material, application of electric connections by soldering (for example, dip soldering).

In electronics, use may, for example, be made of external noble-metal layers manufactured in accordance with the invention in conjunction with one or more of the aforesaid aftertreatments for the manufacture of printed wirings, printed circuits, screening grids, switches and other component parts.

Substantially, all non-metallic, electrically nonconductive support materials, which are, as such, not quite accessible for the various baths for after-treatment may, frequently with the aid of known methods, be rendered hydrophilic to some extent, at least superficially, which suffices, either by given chemical surface treatments or by applying a thin, slightly hydrophilic coating. For example, polystyrene, polyacrylate, bakelite and various other high-polymer products may be rendered accessible for a surface treatment with chlorosulphonic acid (T. Westermark, Acta Chem. Scand. 6, 1194-1199 (1952)). Cellulose esters, polyvinyl acetate and -chloride and so on may be rendered suitable by superficial saponification; glass may be provided by a chemical surface treatment or by coating with a thin layer of silica gel (F. L. Burmistrow, Phot. Journ. 76, 452-459, 1936). Gelatin, regenerated cellulose, paper, wood, polyvinyl alcohol and so on may be used without the need for further means.

If a slightly hydrophylic coating is used, the mercurous compound or the agent capable of reacting with the mercurous compound in the presence of water while separating out mercury can be absorbed directly therein.

#### EXAMPLE I

75 Strips of superficially saponified cellulose tri-acetate

foil were impregnated for two minutes in aqueous solutions of the agents indicated in the first column of Table I, all of which are capable of reacting with a mercurous compound in the presence of water, while separating out metallic mercury. The employed concentrations of these substances in the impregnation liquids are also indicated in the said table. The strips are then wiped off and dried in air at room temperature with the exception of the strips impregnated with sodium sulphite, which are dried in a nitrogen atmosphere. Then the strips are dipped, for a few seconds, in an aqueous solution containing, per litre, 0.005 mol of mercurous nitrate and 0.005 mol of nitric acid. Then they were washed, for 10 sec., in distilled water and, for 10 min., treated in an intensifying bath containing 0.5 g. of metol, 2 g. of citric acid and 0.2 g. of silver nitrate in 100 g. of distilled water. Finally, the strips were again washed in water and dried in air. In Table I a sign + indicates that external, electrically conductive silver layers were obtained on the strips with an electric resistance of not more than  $10^4$  ohm per square. The sign — indicates that no external, electrically conductive silver layers according to the invention were obtained, so that the concentrations concerned cannot be used for the activation of the strips.

Table I

| Agents                                                                  | Concentration: mol/litre |       |       |       |      |     |
|-------------------------------------------------------------------------|--------------------------|-------|-------|-------|------|-----|
|                                                                         | 0.003                    | 0.006 | 0.012 | 0.025 | 0.05 | 0.1 |
| $\text{Na}_2\text{CO}_3$                                                | —                        | +     | +     | +     | +    | —   |
| $\text{Na}_2\text{SO}_3$                                                | —                        | +     | +     | +     | +    | —   |
| $\text{Na}_2\text{S}_2\text{O}_3$                                       | —                        | —     | +     | +     | —    | —   |
| KCNS                                                                    | —                        | —     | —     | +     | +    | +   |
| $\text{S}=\text{C}\begin{cases} \text{NH}_2 \\ \text{NH}_2 \end{cases}$ | —                        | —     | —     | +     | +    | +   |
| $\text{NaNO}_2$                                                         | —                        | —     | —     | —     | +    | —   |
| $\text{Na}_2\text{S}$                                                   | —                        | —     | —     | —     | +    | —   |
| KCN                                                                     | —                        | —     | —     | —     | +    | —   |
| $\text{Sn}(\text{BF}_4)_2$                                              | —                        | —     | +     | +     | +    | —   |

Instead of using the indicated solution for the intensification, but by using one of the following, physical developers containing per 100 g. of distilled water:

- (a) 0.5 g. of metol, 2 g. of lactic acid, 0.1 g. of silver nitrate (developing time 10 min.),
- (b) 1 g. of hydroquinone, 0.2 g. of citric acid and 0.1 g. of silver nitrate (developing time 15 min.),
- (c) 1 g. of hydroquinone, 0.1 g. of lactic acid and 0.1 g. of silver nitrate (developing time 12 min.),
- (d) 0.5 g. of pyrogallol, 1 g. of citric acid, 0.1 g. of silver nitrate (developing time 15 min.),

or a silver-depositing solution obtained by mixing 20 parts by volume of the solution 1, 5 parts by volume of the solution 2 and 1.1 parts by volume of the solution 3, which solutions have the following compositions.

Solution 1: 1 g. of silver nitrate, 2.5 g. of ammonium nitrate, 100 g. of distilled water,

Solution 2: 1.6 g. of sodium hydroxide and 100 g. of distilled water,

Solution 3: 1.25 g. of hydrazine sulphate and 100 g. of distilled water;

qualitatively corresponding results are obtained.

## EXAMPLE II

In the manner described in Example I (strips of the support material referred to therein were treated with aqueous solutions of sodium thiosulphate with the concentrations indicated in Table II. After wiping off and drying, the strips were immersed, for a few seconds, into one of the mercurous nitrate solutions with the concentrations indicated in the Table. These solutions were produced by diluting with distilled water a standard solution containing, per litre, 0.05 mol of mercurous nitrate and 0.05

mol of nitric acid. The further treatment of the strips was similar to that referred to in Example I. Table II indicates the results. The signs have the same meanings as those of Table I.

Table II

| Cone. $\text{Hg}_2(\text{NO}_3)_2$<br>mol/litre | Concentration $\text{Na}_2\text{S}_2\text{O}_3$ in mol/litre |       |       |       |       |      |
|-------------------------------------------------|--------------------------------------------------------------|-------|-------|-------|-------|------|
|                                                 | 0.0015                                                       | 0.003 | 0.006 | 0.012 | 0.025 | 0.05 |
| 0.005                                           | —                                                            | —     | —     | +     | +     | +    |
| 0.0025                                          | —                                                            | —     | +     | +     | +     | +    |
| 0.0012                                          | —                                                            | +     | +     | +     | +     | +    |
| 0.0006                                          | —                                                            | +     | +     | +     | +     | +    |
| 0.0003                                          | —                                                            | +     | +     | +     | +     | +    |

An addition of, for example, citric acid to the mercurous nitrate solution for example 0.1 mol to the solution containing the 0.005 mol of mercurous nitrate and 0.005 mol of nitric acid per litre results in an improved gloss of the final silver layer.

## EXAMPLE III

Table III relates to strips of a superficially saponified cellulose tri-acetate foil treated in the manner described in Example I with the exception that, after impregnation in the solution of the agents capable of reacting with a mercurous compound in the presence of water, while separating out metallic mercury, the strips were wiped off but dipped without intermediate drying in the solution of mercurous nitrate. The signs of Table III have the same meanings as those of the preceding Example. A comparison of results of Table III with those of Table I shows that the omission of the drying process results in that, as a rule, materially higher concentrations of the first activating solution are required than in the case of drying.

Table III

| Agent                             | Concentration, mol/litre |       |      |     |     |     |
|-----------------------------------|--------------------------|-------|------|-----|-----|-----|
|                                   | 0.012                    | 0.025 | 0.05 | 0.1 | 0.2 | 0.4 |
| $\text{Na}_2\text{CO}_3$          | —                        | —     | —    | —   | —   | —   |
| $\text{Na}_2\text{SO}_3$          | —                        | —     | —    | —   | +   | +   |
| $\text{Na}_2\text{S}_2\text{O}_3$ | —                        | —     | +    | +   | —   | —   |

## EXAMPLE IV

Strips of the support material of Example I were dipped for two minutes in an aqueous solution containing per litre 0.005 mol of mercurous nitrate and 0.005 mol of nitric acid. Immediately after the strips had been wiped off, they were treated, for two seconds, with solutions of sodium thiosulphate with the concentrations indicated in Table IV. After washing in distilled water, the strips were treated with metol-citric acid developer of Example I. Finally, the strips were washed in water and dried. The results are indicated in Table IV.

Table IV

| Concentration $\text{Na}_2\text{S}_2\text{O}_3$ ,<br>mol/litre | 0.00035 | 0.0007 | 0.0015 | 0.003 | 0.006 |
|----------------------------------------------------------------|---------|--------|--------|-------|-------|
|                                                                | —       | +      | +      | —     | —     |
| —                                                              | —       | +      | +      | —     | —     |

## EXAMPLE V

Strips of the support material of Example I were dipped, for two minutes, in aqueous solutions containing, per litre, 0.004–0.008–0.016 and 0.032 mol of sodium carbonate and sodium thiosulphate respectively. After wiping off and drying the rear side of the support was covered with a lacquer layer. Subsequently, the strips were dipped, for a few seconds, in the mercurous nitrate solution of Example IV. After washing in distilled water, for a short time, the strips were intensified, for 10 minutes, in a physical developer obtained by dissolving in distilled water: metol

(0.025 mol/litre), citric acid (0.1 mol/litre) and silver nitrate (0.01 mol/litre).

Finally the strips were washed in water and dried in air. The electric resistance values of the external silver layers on the strips activated with the aid of sodium carbonate varied between 130 and 500 ohms per square. After a thermal treatment at 150° C. for one hour, these values had dropped to about 0.25 ohm per square. The resistance values of the silver layers on the strips activated with the aid of sodium thiosulphate varied between 170 and 1100 ohms per square. These values dropped by the said thermal treatment of 0.25–0.6 ohm per square.

#### EXAMPLE VI

Strips of the support material of Example I were dipped for two minutes in one of the following aqueous solutions:

- (A) Thiourea (0.1 mol/litre),
- (B) Sodium thiosulphate (0.03 mol/litre),
- (C) Potassium thiocyanate (0.05 mol/litre).

After wiping off and drying in open air the strips were dipped, for a few seconds, in the mercurous nitrate-nitric acid solution of Example IV. After washing in distilled water, the strips treated with the solutions (A) and (B) were intensified in the physical developer of Example V, whereas the strip treated with the solution (C) was intensified in the metol-citric acid developer of Example I. The developing time was, in all cases, 10 minutes. Finally, the strips were washed in water and dried. The external silver layer on the strip obtained with the solution (A) had an electric resistance of 160 ohms per square, which dropped to 0.4 ohm per square after a treatment at 120° C. for two hours. The silver layer on the strip treated with solution (B) had a resistance of 180 ohms per square which dropped to 0.25 ohm per square by a chemical after-treatment for 2 minutes with a solution of potassium chloride (0.1 mol per litre). By using solutions of sodium bromide, sodium iodide, sodium thiosulphate, sodium sulphite, sulphuric acid, potassium hydroxide, potassium thiocyanate or sodium sulphide instead of the KCl solution material reductions in the original resistance values may be obtained. The silver layer on the strip treated with solution (C) had a resistance of 180 ohms per square. This value was reduced to 13 ohms per square by rubbing with a plug of cottonwool. A further piece of the layer was subjected to a thermal after-treatment at 150° C. for one hour. Then the resistance amounted to 0.7 ohm per square.

#### EXAMPLE VII

An external silver layer on cellulose tri-acetate, obtained in the manner described in Example VI by activation with thiourea and mercurous nitrate, was electrolytically intensified with a few microns of copper by using an aqueous copper-deposition bath of the following composition:

Copper sulphate (5H<sub>2</sub>O) (200 g. per litre),  
Concentrated sulphuric acid (50 g. per litre),  
Phenolsulphonic acid sodium (0.5 g. per litre).

The current density was 5 a./dm.<sup>2</sup> and the time of copper deposition was 2 min. This copper layer was then covered electrophoretically with a layer of aluminum oxide by using a suspension of 10% of alundum in methanol with a field intensity of 37.5 v./cm. for 6 sec. and a current of 70 ma.

#### EXAMPLE VIII

Unilaterally white, woodfree litho-paper was dipped, for 30 sec., on one side in an aqueous solution containing per litre 0.032 mol of sodium thiosulphate. After wiping off, blotting between filter paper, and drying in air, the paper was dipped for a few seconds in the mercurous nitrate-nitric acid solution of Example IV. After washing in distilled water, the layer of mercury germs obtained by activation was intensified in the physical developer of Example V. Finally, the paper with the external silver

layer was washed in water and dried in air. The electric resistance of the silver layer amounted to 500 ohms per square, which value dropped to 7 ohms per square, after a treatment at 150° C. for one hour.

#### EXAMPLE IX

On the support material of Example VIII, there was stamped the desired pattern with the aid of a rubber stamp. The rubber stamp was wetted by means of an inking pad with a 0.05 mol solution of sodium carbonate in water. The sodium carbonate solution had been rendered slightly viscous with the aid of a thickening agent. The activation and the intensification of the mercury germ layer took place in the manner described in Example VIII. By this means there was obtained on the paper an external, electrically conductive silver pattern.

#### EXAMPLE X

An external silver layer formed on the support material of Example I in the manner described in Example VIII was covered with a uniform layer of "Kodak Photoresist" by pouring it out or spraying it. After drying in air, the light-sensitive layer was exposed, for 5 min. behind a pattern (line grid) with the aid of a high-pressure mercury-vapour lamp of 500 w. at a distance of about 50 c.m.s. After the exposure, the layer was "developed" with "Kodak Photoresist Developer" or with trichloroethylene. Then, the mask thus obtained was hardened by treating it at 150° C. for about 10 min. The uncovered portions of the silver layer were then plated with copper for 15 minutes with a current density of 4 a./dm.<sup>2</sup> in an electrolytic bath containing 20% by weight of copper sulphate (5H<sub>2</sub>O) and 6% by weight of sulphuric acid in distilled water. After the mask was removed, the non-plated silver layer was removed by etching. If desired, the metal layer may finally be provided with a protective lacquer layer or with a protective layer of thermo-hardening or thermo-plastic material. In this manner, screening grids may be manufactured.

While we have described our invention in connection with specific embodiments and applications, other modifications thereof will be readily apparent to those skilled in this art without departing from the spirit and scope of the invention as defined in the appended claims.

What is claimed is:

1. A method of producing a permanently adhering external, electrically conductive silver layer on a non-metallic, electrically non-conductive support, at least the surface of said support being hydrophilic, comprising the steps of applying to said support a mercurous compound, water and a compound capable of converting said mercurous compound in the presence of water to free metallic mercury thereby forming a barely visible, at least partially external germ layer of mercury metal on said support, said compound capable of converting said mercurous compound being selected from the group consisting of compounds that reduce mercurous compounds to free mercury metal and compounds that form free mercury metal from mercurous compounds by a disproportionating reaction, said mercury germ layer extending at least partially into the hydrophilic portion of said support, and then treating said mercury germ layer on said support with a silver metal intensifying bath, said bath comprising an aqueous solution of a water soluble silver compound and a water soluble reducing agent for said silver compound to thereby cause a visible, permanently adhering, electrically conducting silver layer to be deposited on said mercury germ layer on said support.

2. The method of claim 1 wherein the mercury germ layer is formed by treating the support in succession first with an aqueous solution of a water soluble mercurous compound and then with an aqueous solution of a water soluble compound capable of converting said mercurous compound to free metallic mercury.

3. The method of claim 1 wherein the compound

capable of converting the mercurous compound is a compound which reduces the mercurous compound to free mercury metal.

4. The method of claim 1 wherein the compound capable of converting the mercurous compound is a compound which converts the mercurous compound into a mercuric compound and free mercury metal by a disproportionating reaction.

5. The method of claim 4 wherein the compound capable of converting the mercurous compound is introduced into the support surface prior to the addition of an aqueous solution of the mercurous compound and this aqueous solution contains, in addition to the mercurous compound an organic hydroxy acid selected from the group consisting of citric acid, tartaric acid, glycolic acid, glycerol acid and malic acid.

6. The method of claim 1, wherein the resultant silver layer is treated with an aqueous solution of at least one water soluble compound yielding in solution an ion selected from the group consisting of the chloride, bromide, iodide, thiocyanate, cyanide, sulfide, sulfite, thiosulfide, hydroxyl and hydrogen ions.

7. The method of claim 6, wherein the ion yielding compound is selected from the group consisting of non-oxidizing acids and acid salts.

8. The method of claim 1 wherein the electrical conductivity of the silver layer is increased by heating said layer to a temperature of at least 80° C.

5 9. The method of claim 1 wherein the electrical conductivity of the silver layer is increased by the electrolytic deposition of additional metal on said silver layer.

10 10. The method of claim 1 wherein the electrical conductivity of the silver layer is increased by mechanically polishing said silver layer.

References Cited by the Examiner

UNITED STATES PATENTS

|           |       |                |         |
|-----------|-------|----------------|---------|
| 168,442   | 10/75 | Worthen et al. | 204—20  |
| 641,709   | 1/00  | Legate         | 204—33  |
| 2,195,231 | 3/40  | Weder          | 204—40  |
| 2,906,682 | 9/59  | Fahnoe et al.  | 204—181 |
| 2,940,018 | 6/60  | Lee            | 204—15  |

FOREIGN PATENTS

|            |      |                |
|------------|------|----------------|
| 20 509,965 | 7/39 | Great Britain. |
|------------|------|----------------|

JOHN H. MACK, Primary Examiner.

JOSEPH REBOLD, Examiner.